

## UNITED STATES PATENT OFFICE

2,135,630

## METHOD OF PRODUCING FERRO-MOLYBDENUM

John D. Sullivan and Dimitry Niconoff, Columbus,  
Ohio, assignors, by mesne assignments, to Kennecott Copper Corporation, New York, N. Y., a corporation of New York

No Drawing. Application October 15, 1937,  
Serial No. 169,234

12 Claims. (CL. 75—21)

Our invention relates to a method of producing ferromolybdenum. It has to do, more particularly, with the production of ferromolybdenum from molybdenite,  $MoS_2$ , concentrates containing appreciable amounts of copper.

Many of the cupriferous ores of the United States contain appreciable amounts of molybdenum in the form of the mineral molybdenite,  $MoS_2$ . Molybdenum can be recovered from these ores by concentration processes but frequently a considerable amount of copper minerals is present in the molybdenite concentrates. This is especially true if a high recovery of molybdenite is desired. The accompanying copper is usually in the form of sulphide which may, for example, be covellite, chalcocite, bornite, chalcopyrite, enargite, tetrahedrite, tennantite or other sulphide or sulphide mineral. No definite limits can be given for the percentages of molybdenite and copper in concentrates because these depend in part on the method of concentration employed, and on the nature of mineral association. Under some conditions nearly pure molybdenite may be obtained while again the molybdenum content of concentrates may be 25 per cent or even lower. The copper may vary from 3 or 4 per cent to 12 or 15 per cent or even higher. In some cases the copper content may be lower than 3 per cent.

In the prior art, success has been had in producing ferromolybdenum from high grade products containing small amounts of copper and other impurities. However, to the best of our knowledge, no practical processes have been developed for economically producing ferromolybdenum from low-grade products containing appreciable amounts of copper and other impurities. For many purposes, the copper content of ferromolybdenum should be low and those methods hitherto utilized for producing ferromolybdenum from high grade products containing small amounts of copper and other impurities have not been economically applicable to the production of low-copper ferromolybdenum from copper-bearing molybdenite concentrates.

One of the objects of this invention is to provide a method for producing a low-copper ferromolybdenum from molybdenite concentrates containing appreciable percentages of copper.

Another object of this invention is to provide a method for producing a low-copper ferromolybdenum from molybdenite concentrates containing appreciable percentages of copper and, at the same time, to produce a copper matte which subsequently can be treated in a copper smelter.

A further object of this invention is to provide a method for producing ferromolybdenum which will be relatively simple and inexpensive.

Other objects will appear in the description following and in the appended claims.

In its preferred form, our invention contemplates smelting of sulphide concentrates or ores containing molybdenite, copper, and other ingredients usually found in concentrates and ores in such a manner that the mass will develop three distinct layers, namely, a slag, a matte and a metal. Normally, the slag will contain the usual impurities and will be low enough in molybdenum to discard. The matte will contain most of the copper and will be low in molybdenum, so that it can be readily treated for the recovery of copper in a copper smelter. The metal will be ferromolybdenum containing copper in amounts which, though appreciable, will not be too high for most purposes for which the ferromolybdenum is to be used.

The percentage of sulphur present during the period of fusion in the smelting step of our process is an important factor in the success of such process. If too little sulphur is present at this time, too much of the copper will tend to combine with the ferromolybdenum and if too much sulphur is present at such time part of the molybdenum will enter the matte together with the copper and iron which normally will be the principal metallic ingredients thereof. As a matter of fact, the sulphur content at the time of fusion may be so high that the product will be practically a single mass substantially devoid of the separate layers which we desire to attain.

The desired sulphur content of the mass during the fusion step may be attained in several ways. It will depend partly on the amounts of molybdenum, copper, iron and other ingredients in the concentrates or ores. It will also depend partly on the type of furnace used in the smelting operation, since some furnaces tend to eliminate as vapor a larger portion of the sulphur than others. It is not feasible to give the exact ranges of sulphur content desired, since these will vary with certain types of concentrates or ores. The important thing is that the sulphur content during the fusion step be within such a range that fusion will result in the formation of substantially distinct layers, one layer being slag with a low percentage of molybdenum therein, another layer being matte and containing most of the copper with very little molybdenum and the third layer being ferromolybdenum wherein the copper content is not too high.

With most of those sulphide concentrates which we have used to date, the sulphur content has been high and, in these cases, we have found it desirable to roast these concentrates or ores to lower the sulphur content to a predetermined value. As indicated above, the sulphur content of the roasted material depends on the amounts of molybdenum, copper, iron, and other ingredients in the concentrates or ores, and on the type of furnace to be used in subsequent melting operations. It may, for example, vary from 5 to 15 per cent, but we do not wish to limit ourselves to this range because in a certain type of concentrates or ores and in certain furnaces these limits may be exceeded. Those skilled in the art can choose a suitable method of roasting. For many purposes, we prefer sintering. However, it should be understood that when we use the term roasting, we intend to include sintering, nodulizing and similar processes.

In the preferred form of our invention, the roasted ore is mixed with sufficient lime or other suitable flux to form a slag with impurities in the ore product and with ingredients of the reducing agent used in a subsequent step. The lime or other flux may be mixed with the concentrates before roasting.

The roasted product and lime or other suitable flux are smelted in a suitable furnace, for example an electric furnace, with iron and a suitable reducing agent to produce a slag, a matte, and a metal. The reducing agent in the charge may be a carbonaceous reducing agent such as coal or coke, or it may be an agent such as silicon or ferrosilicon, or a combination of both types. The amount of iron added will depend on the grade of ferromolybdenum to be produced and on the amount of iron in the ore product. The iron may be in the form of cast iron or steel, for example, scrap, or iron ore may be used, in which case sufficient reducing agent must be present to reduce the iron ore to metal. If sufficient reducing agent is used, the slag will be low enough in molybdenum to discard. The matte will contain most of the copper and will be low in molybdenum. It can be treated for recovery of copper in a copper smelter. The metal will be ferromolybdenum containing an appreciable amount of copper, but for most purposes the copper content is not too high. For many purposes the sulphur content of the ferromolybdenum is too high; so it is treated with a desulphurizing slag, which for example may be a high lime slag. If the desulphurizing slag is sufficiently reducing, the molybdenum content will be low enough to permit discarding it, but if it contains an appreciable amount of molybdenum it can be returned as part of the charge in the initial smelting operation. We have been able to reduce the copper content of ferromolybdenum to below 1.5% by this procedure.

It is obvious, of course, that if any matte-forming constituents other than copper are present they will likewise be separated in the matting operation. The process, therefore, in its broadest sense involves removal of matte-forming constituents from molybdenum products by a smelting process.

As a modification of this method, in some instances it may be unnecessary to roast the concentrates. This is true if iron ore is used as a source of iron. Also, in some instances it is possible to use a higher sulphur content in the charge although additional lime will be used either in the charge to slag the additional sulphur or in

the desulphurizing slag used to refine the ferromolybdenum.

Important features are that sufficient flux should be present to slag the ingredients to be removed from the charge and sufficient sulphur should be present to form a copper matte. It is obvious that part of the concentrates may be roasted even to a dead-roasted condition and the sulphur in the charge brought up with raw concentrates. Likewise, it may be possible to dead-roast all the concentrates and add sulphur as a sulphur-bearing material, for example pyrite.

Although the product made by the smelting procedure outlined will be in a marketable form suitable for most commercial uses, in some instances it will be necessary to produce a ferromolybdenum with still lower copper content. This invention is also concerned with making such a product by the following procedure.

After the initial smelting step, the slag and mate are removed. The next step comprises forming a matte to remove most of the copper remaining in the metal. As a first step it is usually desirable to increase the sulphur content of the metal, preferably to about 5 per cent or even higher if the metal does not already contain this amount. This can be done by adding a sulphide-containing material, for example, raw concentrates or pyrite. If raw concentrates are used, sufficient lime or other flux should be used to form a slag with the impurities therein. In either case some matte will be formed, and if concentrates are used some slag will also be formed, which should be low enough in molybdenum to reject. The matte formed when concentrates are used probably will contain enough molybdenum to justify returning it to the original smelting furnace as part of the initial charge. If pyrite is used for sulphurizing, the matte formed in this operation will be low in molybdenum, and it is not necessary to remove it before proceeding with the next operation. After sulphurization, the next step is adding pyrite or similar matting agent to matte off most of the copper still remaining in the metal.

To reduce the copper content still lower the metal is treated with ferromanganese or with manganese ore and a suitable reducing agent to form a manganese-copper matte. It is not necessary to skim the matte between the pyrite and manganese treatments. Of course, skimming the pyrite matte before addition of manganese is optional. The composite or individual mattes will be low in molybdenum and can be treated for their copper content in a copper smelter. The ferromolybdenum will be low in copper, but will contain an appreciable amount of sulphur; so it is treated with a basic desulphurizing slag. The metal after the desulphurizing treatment will be low in sulphur. The copper content will be 0.7 per cent or less, and may be lower than 0.5 per cent. The desulphurizing slag, if reducing, may be low enough in molybdenum to discard, or if it contains molybdenum, it can be added as part of the charge in the initial smelting step. It is obvious, of course, that should any product outlined above for removal from the system be too high in molybdenum to discard it can be returned to the circuit to recover the molybdenum therein.

In the above matting operation, in which the copper content of ferromolybdenum is reduced by means of a manganese-containing material, we have found that other matting agents are also effective in lowering the copper content of the ferromolybdenum. We have, for example, used

ferrochromium, aluminum, and ferrosilicon. Because of their availability and relatively low cost, we ordinarily prefer to use manganese products.

While the process has been carried out on numerous products in various furnaces two examples will be given to illustrate the principal features of the invention. Concentrates of the following chemical analyses was used:

| 10                                  | Ingredient | Per cent |
|-------------------------------------|------------|----------|
| Mo.                                 | 30.2       |          |
| Cu.                                 | 10.6       |          |
| Fe.                                 | 10.0       |          |
| S.                                  | 28.2       |          |
| 15 Al <sub>2</sub> O <sub>3</sub> . | 3.3        |          |
| SiO <sub>2</sub> .                  | 12.6       |          |
| MgO.                                | 2.0        |          |

Example 1.—A charge of 66 lbs. roasted calcines containing 5 per cent of S and 8.3 per cent each of coal and CaO, 15.5 lbs. raw concentrates, 10.5 lbs. iron shavings, and 10.5 lbs. coal was smelted in an electric furnace. The resultant metal after removal of slag and matte contained 46.8 per cent of Mo and 1.4 per cent of Cu.

Example 2.—Concentrates were sintered with lime to yield a product containing 25.6 per cent of Mo, 12.7 per cent of S, and 10 per cent of CaO. A mixture of 540 lbs. sinter, 125 lbs. boiler plate punchings, and 75 lbs. coke was smelted in an electric furnace. After the slag and matte were removed, 70 lbs. of concentrates containing 82 per cent of MoS<sub>2</sub> was added. The matte and slag were removed, and 15 lbs. pyrite added, and after reaction between pyrite and metal 15 lbs. high-carbon, 80 per cent Mn, ferromanganese was added. The matte was removed, and the metal treated with a high lime slag. The final metal analyzed as follows:

| 40  | Ingredient | Per cent |
|-----|------------|----------|
| Mo. | 61.3       |          |
| Cu. | 0.7        |          |
| S.  | 0.14       |          |
| Mn. | 0.05       |          |
| P.  | 0.05       |          |
| Si. | 0.06       |          |
| As. | Trace      |          |
| C.  | 2.2        |          |

The above examples are illustrative only, and other grade concentrates can be used, and any of the alternative procedures can be employed. For example, ferrosilicon can be used instead of coke as the reducing agent and sulphurizing may be effected by pyrite instead of concentrates. Obviously the step of treatment with manganese may be omitted if the copper content is low enough in the ferromolybdenum for its contemplated use.

It will be seen from the above that we have provided a novel method which is of great importance to the metallurgical industry because it is a simple and inexpensive method by which ferromolybdenum suitable for the metallurgical industry can be obtained from low grade products containing appreciable amounts of copper and other materials. Moreover, the amount of copper present in the ferromolybdenum produced can be regulated to render it suitable for any particular purpose for which it is to be utilized. Thus, it will be seen that this invention makes possible the use of concentrates and ore products for the making of ferromolybdenum that have not previously been available because there has

been no simple and economical method for recovering ferromolybdenum from such concentrates and ore products which ferromolybdenum is substantially free from objectionable quantities of copper. It is likewise apparent that our process results in the formation of a matte which contains substantially all of the copper in the concentrates or ores and which can readily be treated in a copper smelter.

In the claims, the term "iron" is intended to include cast iron, ingot iron, steel or iron ore together with a suitable reducing agent. Likewise, the term "concentrates", as used in the claims is intended to include high grade ores which do not require concentration.

Having thus described our invention, what we claim is:

1. The method of making ferromolybdenum from copper-bearing molybdenum-containing material which comprises smelting a charge containing a copper-bearing molybdenum product, a slag-forming flux, a reducing agent, and iron, such charge being further characterized by containing sulphur in selected amount and with the components so proportioned and in such form as to yield slag, matte, and metal consisting primarily of ferromolybdenum, and separating the metal from the slag and matte.

2. The method of making ferromolybdenum from copper-bearing molybdenum-containing materials which comprises smelting a charge containing a copper-bearing molybdenum product, a slag-forming flux, a reducing agent, and iron, such charge being further characterized by containing sulphur in selected amount and with the components so proportioned and in such form as to yield slag, matte, and metal consisting primarily of ferromolybdenum, removing the slag and matte and treating the metal with a desulphurizing slag.

3. The method of making ferromolybdenum from a molybdenum product containing a matte-forming ingredient which comprises smelting a charge containing said molybdenum product, a slag-forming flux, a reducing agent, and iron, such charge being further characterized by containing sulphur in selected amount and with the components so proportioned and in such form as to yield slag, matte, and metal consisting primarily of ferromolybdenum, and separating the metal from the slag and matte.

4. A method of making ferromolybdenum which comprises selecting copper-bearing molybdenite concentrates, adjusting the sulphur content of the concentrates to within a selected range such that a copper matte will be formed during subsequent smelting, smelting said concentrates with a slag-forming flux, iron and a reducing agent to form during fusion a layer of slag, a matte and a metal consisting primarily of ferromolybdenum, and then separating the metal from the slag and matte.

5. The method of making ferromolybdenum from copper-bearing molybdenum-containing material which comprises smelting a charge containing said molybdenum product, a slag-forming flux, a reducing agent, and iron, such charge being further characterized by containing sulphur in selected amount and with the components so proportioned and in such form as to yield slag low in molybdenum, matte, and metal high in ferromolybdenum, and separating the metal from the slag and matte.

6. A method of making ferromolybdenum which comprises smelting partly roasted copper-bear-

ing molybdenite concentrates with iron, a reducing agent, and a flux capable of forming a slag with ingredients in the charge to form a slag, matte and metal, removing the slag and matte, adding additional concentrates and removing the matte formed, adding successively pyrite and one of the group consisting of manganese, ferromanganese, and manganese ore and a reducing agent, removing the matte and treating the metal with 10 a desulphurizing slag.

7. A method of making ferromolybdenum which comprises smelting partly roasted copper-bearing molybdenite concentrates with iron, a reducing agent, and a slag-forming flux, removing the slag 15 and matte formed, and treating the metal with a desulphurizing slag.

8. A method of making ferromolybdenum which comprises smelting partly roasted copper-bearing molybdenite concentrates with iron, a reducing agent, and a slag-forming flux to produce a 20 slag, a matte and a metal, and then removing the slag and the matte.

9. A method of making ferromolybdenum which comprises smelting partly roasted copper bearing molybdenite with iron and a reducing agent to form a matte and metal, removing the matte, adding a sulphide-bearing material to the metal 25

to form a copper-bearing matte, removing the matte, and treating the metal with a slag to reduce the sulphur content.

10. A method of decopperizing ferromolybdenum which comprises adding to copper-bearing ferromolybdenum a sulphurizing agent and one of the group consisting of manganese, ferromanganese, and manganese ore and a reducing agent to remove copper as a manganese-copper matte. 5

11. A method of making ferromolybdenum 10 which comprises smelting partly roasted copper-bearing molybdenite concentrates with iron, a reducing agent, and a flux capable of forming a slag with ingredients in the charge to form a slag, matte and metal, removing the slag and matte, 15 adding a sulphide-bearing material to the metal, adding a matte-forming ingredient to the metal, removing the matte formed, and then treating the metal with a desulphurizing slag.

12. A method of making ferromolybdenum 20 which comprises the step of adding to copper-bearing ferromolybdenum a sulphurizing agent and a matte-forming agent to remove copper as a matte.

JOHN D. SULLIVAN. 25  
DIMITRY NICONOFF.